

# UNITED STATES PATENT OFFICE.

MORRIS FINKELSTEIN, SAMUEL H. FINKELSTEIN, HARRY L. FINKELSTEIN, AND  
NATHAN FINKELSTEIN, OF GREENVILLE, MISSISSIPPI.

## THREAD-COATING COMPOSITION.

1,210,446.

Specification of Letters Patent.

Patented Jan. 2, 1917.

No Drawing.

Application filed August 6, 1915. Serial No. 44,089.

*To all whom it may concern:*

Be it known that we, MORRIS FINKELSTEIN, SAMUEL H. FINKELSTEIN, HARRY L. FINKELSTEIN, and NATHAN FINKELSTEIN, 5 citizens of the United States, residing at Greenville, in the county of Washington and State of Mississippi, have invented certain new and useful Improvements in Thread-Coating Compositions, of which the following is a specification.

This invention relates to a wax composition possessing such properties as enable it to replace both the type of wax and the means for heating the same which are now 15 customarily employed in connection with the operation of shoe and harness machines, for the purpose of coating the thread before stitching.

Practically every modern machine of the 20 character mentioned is equipped with a comparatively costly gas heater attachment for the purpose of softening ordinary wax in order to permit the thread to be drawn through the latter and to have its fibers 25 thoroughly permeated therewith as it necessary for the purpose of stiffening the thread and rendering it more durable. These attachments, however, in addition to their cost are the cause of many inconveniences, 30 such as loss of time, loss of material when the machine is accidentally overheated, the possibility of a dangerous explosion and the frequent injuring of the workman's hands due to a spattering of the melted wax.

The wax composition provided by the 35 present invention overcomes all of these grave objections by providing a wax which is of such a fluid consistency as to permit the thread to be readily drawn therethrough 40 without the previous application of heat to reduce the wax to a molten state. Certain ingredients of the composition act as permanent diluents of the wax until the composition is used to coat the thread body, 45 when the diluents form the permeating vehicle for the wax, later to be naturally evaporated therefrom, after the wax has attained its intimate position with respect to the fibers of the thread body.

50 The above and additional objects which will be hereinafter more specifically treated are accomplished by means of the composition the formation of which is described in the following specification and then more

fully pointed out in the claims which are 55 appended hereto and form a part of this application.

The composition consists essentially in the combination or admixture, by weight, measure, or otherwise, in the requisite proportions and in the manner to be later set forth in particular, of the following three ingredients, viz: white wax, varnish and turpentine.

It has been found by experiments in the 65 reduction of this invention to practice that the ingredients should be mixed in the following proportions to obtain an approximate two pounds of the composition: white wax, one pound, four ounces; four and one-half 70 ounces of any light or clear varnish; and four and one-half ounces of turpentine. In mixing the above ingredients to prepare the composition, a suitable vessel is placed over a gentle flame and the white wax is 75 placed thereinto. When the wax is well melted the vessel is placed in a second and larger vessel which contains a quantity of water adapted to surround the first vessel to prevent explosion by keeping the temperature 80 of the first vessel down to or below that of boiling water. The varnish and turpentine are next entered and the flame is reduced. When the surrounding water in the larger vessel begins boiling, the mixture is 85 stirred for a period of five (5) minutes. After this the composition is set aside to cool, when it will be in readiness for immediate use. This method of melting the white wax and forming an intimate mixture 90 therewith of turpentine and varnish which serve as diluents and permeating vehicles for the wax, obviate the necessity of melting the white wax by means of the dangerous, costly and inefficient gas attachment now 95 customarily employed.

While the foregoing sets forth the ingredients and method of preparing the composition of this invention and designates the ingredients by their best known commercial names, it is understood that ingredients which may be differently named, although possessing the same properties or qualities, are also comprehended by this invention, as well as their equivalents.

100 105

What is claimed is:—

1. A wax composition including as ingredients white wax, turpentine and varnish,

intimately mixed together substantially in or about the proportions set forth and in the manner and for the purpose described.

2. A wax composition consisting of white 5 wax, turpentine, and a clear, light varnish mixed substantially in the proportions set forth and in a manner described.

3. A wax composition comprising an intimate mixture of white wax about 20 parts 10 by weight, turpentine about 5 parts by weight, and 5 parts of a clear, light varnish by weight.

In testimony whereof we affix our signatures in presence of two witnesses.

MORRIS FINKELSTEIN.

SAMUEL H. FINKELSTEIN.

HARRY L. <sup>bis</sup> X FINKELSTEIN.

NATHAN FINKELSTEIN. <sup>mark</sup>

Witnesses:

SOL ROSENBLUM,  
HARRIS BERGER.